

# United States Patent

Becker

[15] 3,639,182

[45] Feb. 1, 1972

[54] **METHOD FOR IMPROVING THE  
EFFECTIVENESS OF A MAGNETIC  
FIELD FOR MAGNETIZING  
PERMANENT MAGNETS**

[72] Inventor: **Joseph J. Becker, Schenectady, N.Y.**

[73] Assignee: **General Electric Company**

[22] Filed: **Mar. 27, 1969**

[21] Appl. No.: **818,465**

[52] U.S. Cl. .... **148/103, 148/108, 252/62.51,  
252/62.63**

[51] Int. Cl. .... **H01f 13/00, H01f 1/10, H01f 1/04**

[58] Field of Search..... **148/100, 101, 103, 108, 102;  
252/62.51, 62.63**

[56] **References Cited**

UNITED STATES PATENTS

|           |         |                        |             |
|-----------|---------|------------------------|-------------|
| 2,482,364 | 9/1949  | Pfleger.....           | 148/108 X   |
| 3,036,008 | 5/1962  | Berge.....             | 252/62.63 X |
| 3,066,355 | 12/1962 | Schloemann et al. .... | 148/103 X   |
| 3,067,140 | 12/1962 | Davis, Jr. ....        | 148/108 UX  |
| 3,113,927 | 12/1963 | Cochardt.....          | 252/62.5    |

|           |         |                     |           |
|-----------|---------|---------------------|-----------|
| 3,117,065 | 11/1964 | Wootten .....       | 148/108 X |
| 3,226,266 | 12/1965 | Jesmont et al. .... | 148/103 X |
| 3,279,959 | 10/1966 | Oshima et al. ....  | 148/103   |
| 3,424,578 | 1/1969  | Strnat et al. ....  | 75/213    |
| 3,428,498 | 2/1969  | Heimke.....         | 148/103 X |

Primary Examiner—Hyland Bizot

Assistant Examiner—G. K. White

Attorney—Charles T. Watts, Paul A. Frank, James M. Binkowski, Frank L. Neuhauser, Oscar B. Waddell and Joseph B. Forman

[57] **ABSTRACT**

A method for increasing the coercive force of a permanent magnet produced by a given magnetizing field. The magnet is subjected to the magnetizing field with the initial position of the magnet being no greater than an angle  $\theta$  of  $\pm 45^\circ$  formed between a predetermined direction of magnetization of the magnet and the direction of the applied magnetizing field. The magnet and/or magnetizing field are moved in at least a single plane through the angle  $\theta$  which can range up to  $\pm 45^\circ$ . Such movement is terminated with the magnet in a position in which its predetermined direction of magnetization is substantially parallel to the direction of the magnetizing field.

10 Claims, 1 Drawing Figure

PATENTED FEB 1 1972

3,639,182



INVENTOR:

JOSEPH J. BECKER,

by Jane M. Binkowski

HIS ATTORNEY

**METHOD FOR IMPROVING THE EFFECTIVENESS OF A MAGNETIC FIELD FOR MAGNETIZING PERMANENT MAGNETS**

The present invention relates generally to the art of making permanent magnets and is more particularly concerned with a novel method for improving the effectiveness of a magnetic field for magnetizing such magnets.

It is generally recognized that the magnetic properties of permanent magnet materials can be enhanced by reducing them to powders. Ordinarily, magnets of such powders are prepared by subjecting them to a magnetic field to orient the particles, compressing the powder and sintering the resulting compacts. The magnetic powder can also be bonded in rubber or plastic to produce flexible permanent magnets having special utility in permanent magnet motors, as magnetic latches, and in many other applications. In some instances, the enhancement of the properties by particle size reduction is offset to a substantial degree by the accompanying decrease in magnetic coercive force. Due to the numerous potential applications of permanent magnets, substantially increasing their coercive force has long been recognized as a desirable objective by those skilled in the art.

I have found that the value of the magnetic coercive force  $H_c$  of permanent magnets, especially magnets of cobalt rare-earth compounds, shows a pronounced dependence on the magnetizing field  $H_m$ . Specifically, magnets formed from permanent magnet material powders, especially powders of cobalt rare-earth compounds, exhibit an unusually large dependence of coercive force on the previously applied magnetizing field. This dependence appears even when the coercive forces have the low values associated with magnets formed from a large particle size material. To develop their best magnetic properties, therefore, the permanent magnets need to be magnetized in as strong a field as possible. The stronger the magnetizing field, however, the greater are the energy requirements for furnishing such a field. In addition, the rate of rise of the coercive force  $H_c$  with the magnetizing field  $H_m$ , in some instances, suggests that sufficiently strong magnetic fields are not presently available to any significant extent to impart the highest coercive force.

I have further discovered that the effectiveness of a given magnetic field used for magnetizing a permanent magnet to increase its coercive force can be very substantially enhanced by causing relative motion between the magnetic field and the body being magnetized, such motion being critical in both extent and kind.

According to the present invention, the relative motion between the magnetizing field and the permanent magnet can be carried out in a number of ways. For example, it can be carried out by selective movement of the magnet in the magnetizing field, by selective movement of the magnetizing field along or by selective movement of the magnet and its magnetizing field. Since the magnetizing field is usually supplied by a large magnet secured in place, the preferred embodiment of the present invention is the selective movement of the magnet in the magnetizing field.

Briefly stated, the preferred embodiment of the present invention comprises subjecting the permanent magnet to a magnetizing field. The initial position of the magnet in the magnetizing field can vary but it should be no greater than at an angle  $\theta$  of  $\pm 45^\circ$ , the angle  $\theta$  being formed between a predetermined direction of magnetization of the magnet and the direction of the applied magnetizing field. For convenience, the magnet can be positioned initially with the angle  $\theta$  having a value of 0, at which position, the predetermined direction of magnetization of the magnet and the direction of the magnetizing field are substantially parallel. The permanent magnet is then moved in the magnetizing field in at least a single plane through the angle  $\theta$  with such angle ranging up to about  $\pm 45^\circ$ . The movement of the magnet in the magnetizing field is terminated with the predetermined direction of magnetization of the magnet substantially parallel to the direction of the magnetizing field.

The process of the present invention is operable with permanent magnets. Such magnets may be anisotropic or isotropic. If the magnet is anisotropic, it has a magnetically preferred spacial direction, i.e., an easy axis of magnetization, and its predetermined direction of magnetization as used herein is generally such magnetically preferred direction. If the magnet is isotropic, its magnetic properties are the same in all spacial directions, and its predetermined direction of magnetization as used herein can be any desired direction.

10 The accompanying figure illustrates one method of carrying out the present invention wherein the magnet was positioned initially with the angle  $\theta$  having a value of 0, i.e., the predetermined direction of magnetization of the magnet was parallel to the direction of the magnetizing field. As shown by the figure, the magnet was moved in a single plane through an angle of  $+45^\circ$ , then  $-45^\circ$ , and then such movement was terminated with the angle  $\theta$  having a value of 0.

In carrying out the process of the present invention, the magnet should not be moved through an angle  $\theta$  greater than  $\pm 45^\circ$  because such movement would tend to cause reversal of the magnetization of those particles whose magnetic axis initially made an angle of more than  $45^\circ$  with the predetermined direction of magnetization of the sample. Although the angle  $\theta$  can have a value less than  $\pm 45^\circ$ , an angle  $\theta$  having a maximum value of  $\pm 45^\circ$  is preferred since it results in most instances in the highest increase in coercive force.

In the instant process, the coercive force can be further improved by movement of the magnet through the angle  $\theta$  in a plurality of planes. For example, movement of the magnet through an angle  $\theta$  of up to  $\pm 45^\circ$  through two perpendicular planes successively further increases the coercive force significantly. Since the angle  $\theta$ , in circumscription, defines a cone, the maximum coercive force is obtained by successively moving the magnet through a number of different planes with the angle  $\theta$  equal to  $\pm 45^\circ$  so that all orientations of the magnet's particles around the cone are covered.

In the process of the present invention, movement of the magnet in the magnetizing field can be carried out manually or mechanically by a number of conventional techniques. The rate of movement of the magnet can vary widely since it is not critical. When the desired movement of the magnet is completed, such movement is terminated with the predetermined direction of magnetization of the magnet substantially parallel to the direction of the magnetizing field. After such magnetization, the coercive force of the magnet is measured.

The particular form of the magnet used in the present process can vary widely and is not critical. The greatest improvement in properties is usually produced with magnets formed from powders of permanent magnet materials. The present process, however, is also operable with permanent magnet materials in bulk form, i.e., those magnets which have never been reduced to particulate form.

55 Representative of the permanent magnet materials useful in the present invention are cobalt-base permanent magnet materials such as  $\text{Co}_2\text{Y}$ ,  $\text{Co}_5\text{Sm}$  and  $\text{Co}_5\text{M}$  wherein M is cerium-rich misch metal. Additional representative materials are the magnetically hard ferrite powders. Typical of these powders are barium ferrite ( $\text{BaO} \cdot 6 \text{Fe}_2\text{O}_3$ ), strontium ferrite ( $\text{SrO} \cdot 6 \text{Fe}_2\text{O}_3$ ) and lead ferrite ( $\text{PbO} \cdot 6 \text{Fe}_2\text{O}_3$ ).

60 Alternatively, the present process can be carried out by moving the permanent magnet in the magnetizing field so that the angle  $\theta$  is increased by increments. Specifically, starting with the angle  $\theta$  having a value of substantially 0, the magnet is moved through an angle  $\theta$  having a value greater than 0 but less than  $45^\circ$ , through successively different planes so that its predetermined direction of magnetization describes a cone around the direction of the magnetizing field  $H_m$ . With each additional movement of the magnet so that a cone is defined, the angle  $\theta$  is increased until it equals  $\pm 45^\circ$ .

In another embodiment of the present process, movement of the magnet in a series of successive planes displaced from each other by a suitable angular increment can be accomplished by rotating the magnet through a suitable angle around

the predetermined axis of magnetization at the completion of each movement in a single plane through the angle  $\theta$ .

The present invention is further illustrated by the following examples.

#### EXAMPLE 1

A cylindrical magnet, about five-sixteenths inch in diameter and three-eighths inch long, was prepared from  $\text{Co}_5\text{Sm}$  powder which had a particle size of about -325 mesh. The powder was pressed while in hexane so that excess fluid leaked out of the die during compression. It was compressed lightly in a magnetic field of 8,000 oersteds to orient the particles along their easy axis of magnetization. The resulting compact was then further compressed outside the magnetic field under a pressure of 80,000 p.s.i. It was then placed in a vacuum to evaporate the hexane and then impregnated with an epoxy resin by means of a differential pressure technique.

The resulting cylindrical article was the test magnet used in a number of runs with a specific magnetizing procedure being used in each run as shown in the following table. For comparison purposes, initially, in each run, this magnet was placed in the same reference state by magnetizing it in a field of 23,600 oersteds as disclosed in the following table.

| Run | Magnetizing Procedure                                                                                                                                                                                                                                                                                                                                                                                                                                                                              | Force<br>(oersteds) | Coercive<br>(oersteds) |
|-----|----------------------------------------------------------------------------------------------------------------------------------------------------------------------------------------------------------------------------------------------------------------------------------------------------------------------------------------------------------------------------------------------------------------------------------------------------------------------------------------------------|---------------------|------------------------|
| 1   | With its easy axis of magnetization aligned with the direction of the magnetic field, i.e., the $0^\circ$ position of the angle $\theta$ , the test magnet was magnetized in a magnetic field of 23,600 oersteds to establish a reference state. It was then magnetized in the opposite direction in a magnetizing field of 15,000 oersteds.                                                                                                                                                       | 2550                |                        |
| 2   | The test magnet was returned to its reference state by magnetizing it in a magnetic field of 23,600 oersteds as in run 1. It was then magnetized in the opposite direction in a magnetizing field of 15,000 oersteds by moving it in the same plane from its $0^\circ$ position through an angle $\theta$ of $45^\circ$ , then back through the same plane, through the $0$ position, through an angle $\theta$ of $-45^\circ$ and back to $0$ position as illustrated in the accompanying figure. | 3290                |                        |
| 3   | The test magnet was magnetized as in run 1.                                                                                                                                                                                                                                                                                                                                                                                                                                                        | 2530                |                        |
| 4   | The entire procedure of run 2 was repeated except that magnetization of the test magnet in the field of 15,000 oersteds was made by moving it through the angle $\theta$ of $\pm 45^\circ$ in two perpendicular planes successively. The test magnet was magnetized as in run 1.                                                                                                                                                                                                                   | 2600                | 5                      |
| 6   | The entire procedure of run 4 was repeated except that magnetization of the test magnet in the field of 15,000 oersteds was made by moving the magnet $\pm 45^\circ$ in four planes at $45^\circ$ to each other.                                                                                                                                                                                                                                                                                   | 4150                |                        |
| 7   | The procedure of run 1 was used except that a magnetizing field of 20,000 oersteds was used instead of 15,000 oersteds.                                                                                                                                                                                                                                                                                                                                                                            | 3850                |                        |
| 8   | The procedure of run 2 was used except that a magnetizing field of 20,000 oersteds was used instead of 15,000 oersteds.                                                                                                                                                                                                                                                                                                                                                                            | 4750                |                        |
| 9   | The procedure of run 4 was used except that a magnetizing field of 20,000 oersteds was used instead of 15,000 oersteds.                                                                                                                                                                                                                                                                                                                                                                            | 5000                |                        |
| 10  | The procedure of run 6 was used except that a magnetizing field of 20,000 oersteds was used instead of 15,000 oersteds.                                                                                                                                                                                                                                                                                                                                                                            | 5150                |                        |
| 11  | The procedure of run 1 was used except that a magnetizing field of 29,000 oersteds was used instead of 15,000 oersteds.                                                                                                                                                                                                                                                                                                                                                                            | 5400                |                        |
| 12  | The procedure of run 6 was used except that a magnetizing field of 29,000 oersteds was used instead of 15,000 oersteds.                                                                                                                                                                                                                                                                                                                                                                            | 5400                |                        |

The above table illustrates the significant increase in coercive force which can be produced in a cobalt rare-earth permanent magnet material by the method of the present invention. Specifically, runs 2, 4, 6, 9 and 10 illustrate the process of the present invention. Run 2 illustrates movement of the test magnet in one plane with the angle  $\theta$  being  $\pm 45^\circ$  and shows a significantly higher coercive force than that produced in control runs 1 and 3 where the strength of the magnetizing

field was the same but the test magnet was stationary. Runs 4 and 6 show an even higher coercive force than run 2 due to movement of the test magnet in a greater number of planes. Runs 11 and 12 illustrate that when the magnetizing field applied is high enough, the coercive force of the test magnet remains unchanged by relative motion between the magnet and the magnetizing field.

The present process is operable, therefore, with any permanent magnet material in the range in which the coercive force depends on the magnetizing field, in which range the effectiveness of a given magnetizing field can be enhanced. As a result, permanent magnets with high coercive forces are available for much wider use than has been heretofore practicable since the high energy requirements of large magnetizing fields are eliminated.

#### EXAMPLE 2

In this example, a commercial oriented strontium ferrite cylindrical magnet about one-half inch in diameter and about five-sixteenths inch long was used. The magnet had been oriented along its easy axis of magnetization.

After stationary magnetization in a field of 10,000 oersteds, with its easy axis of magnetization substantially parallel, i.e., aligned with the direction of the magnetizing field, i.e., with the angle  $\theta$  having a value of  $0^\circ$ , the magnet had a coercive force of 3,430 oersteds. It was then magnetized in the same field by moving it from its position of alignment with the direction of the field, i.e., the  $0^\circ$  position of  $\theta$ , through an angle  $\theta$  of  $\pm 45^\circ$  in four planes, with each plane at  $45^\circ$  to each other, and terminating such movement with the easy axis of magnetization substantially parallel with the direction of the magnetizing field. After such magnetization, its coercive force was unchanged indicating that the magnetizing field was so high that coercive force no longer varied with relative motion.

In its position of alignment with the field, i.e., with its easy axis of magnetization parallel with the direction of the field, the strontium ferrite magnet was then magnetized in the opposite direction in a magnetic field of 5,000 oersteds. After such magnetization, its coercive force was determined to be 3,000 oersteds. It was then magnetized in the same field by moving it from its position of alignment, through an angle  $\theta$  of  $\pm 45^\circ$  in four planes, with each plane being  $45^\circ$  to each other and terminating such movement with the easy axis of magnetization substantially parallel with the direction of the magnetizing field. After such magnetization, the coercive force was determined to be 3,350 oersteds.

#### EXAMPLE 3

The procedure of this example was the same as that set forth in example 2 except that a commercial oriented barium ferrite magnet was used. The magnet had been oriented along its easy axis of magnetization.

After stationary magnetization in a field of 10,000 oersteds with its easy axis of magnetization substantially parallel, i.e., aligned, with the direction of the magnetizing field, i.e., with the angle  $\theta$  having a value of  $0^\circ$ , the magnet had a coercive force of 2,400 oersteds. It was then magnetized in the same field by moving it from its position of alignment with the direction of the field through an angle  $\theta$  of about  $\pm 45^\circ$  in four planes, with each plane at  $45^\circ$  to each other and terminating such movement with the easy axis of magnetization substantially parallel with the direction of the magnetizing field. After such magnetization, its coercive force was unchanged, indicating that the magnetizing field was so high that coercive force no longer varied with relative motion.

In its position of alignment with the magnetizing field, i.e., with its easy axis of magnetization parallel with the direction of the field, the barium ferrite magnet was then magnetized in the opposite direction in a magnetizing field of 5,000 oersteds. After such magnetization, its coercive force was determined to be 2,130 oersteds. It was then magnetized in the same field by moving it from its position of alignment through an angle  $\theta$

of about  $\pm 45^\circ$  in four planes, with each plane being  $45^\circ$  to each other, and terminating such movement with the easy axis of magnetization substantially parallel with the direction of the magnetizing field. After such magnetization, the coercive force was determined to be 2,380 oersteds.

What is claimed is:

1. A method for increasing the coercive force of a permanent magnet in a given magnetizing field which comprises subjecting the magnet to the magnetizing field, the initial position of said magnet in said magnetizing field being no greater than an angle  $\theta$  of  $\pm 45^\circ$ , the angle  $\theta$  being formed between a predetermined direction of magnetization of the magnet and the direction of the applied magnetizing field, causing relative motion between the magnet and the magnetizing field in at least a single plane through the angle  $\theta$  with said angle  $\theta$  ranging up to  $\pm 45^\circ$ , and ending such movement with the predetermined direction of magnetization of the magnet substantially parallel to the direction of the magnetizing field.

2. A method for increasing the coercive force of a permanent magnet in a given magnetizing field which comprises subjecting the magnet to the magnetizing field, the initial position of said magnet in said magnetizing field being no greater than an angle  $\theta$  of  $\pm 45^\circ$ , the angle  $\theta$  being formed between a predetermined direction of magnetization of the magnet and the direction of the applied magnetizing field, moving the permanent magnet in the magnetizing field in at least a single plane through the angle  $\theta$  with said angle  $\theta$  ranging up to about  $\pm 45^\circ$ , and ending such movement of the magnet in the magnetizing field with the predetermined direction of magnetization of the magnet substantially parallel to the direction of the magnetizing field.

3. A method according to claim 1 wherein said predetermined direction of magnetization is the magnetically preferred direction of magnetization.

4. A method according to claim 2 wherein the initial position of said magnet in said magnetizing field is at an angle  $\theta$  of substantially  $0^\circ$ .

5. A method for increasing the coercive force of a permanent magnet in a given magnetizing field which comprises subjecting the magnet to the magnetizing field, the initial position of said magnet in said magnetizing field being no greater than an angle  $\theta$  of  $\pm 45^\circ$ , the angle  $\theta$  being formed between a predetermined direction of the magnet and the direction of the applied magnetizing field, moving the permanent magnet in the magnetizing field in a plurality of planes through the angle  $\theta$  with said angle  $\theta$  ranging up to about  $\pm 45^\circ$ , and ending such movement of the magnet in the magnetizing field with the predetermined direction direction of magnetization of the magnet substantially parallel to the direction of the magnetizing field.

6. A method according to claim 1 wherein said permanent magnet material is a cobalt rare-earth compound.

7. A method according to claim 6 wherein said cobalt rare-earth compound is a member of the group consisting of  $\text{Co}_5\text{Y}$ ,  $\text{Co}_5\text{Sm}$  and  $\text{Co}_5\text{M}$  wherein M is cerium-rich misch metal.

8. A method according to claim 1 wherein said permanent magnet material is a magnetically hard ferrite.

9. A method according to claim 8 wherein said magnetically hard ferrite is selected from the group consisting of barium ferrite, strontium ferrite and lead ferrite.

10. A method for increasing the coercive force of a permanent magnet in a given magnetizing field which comprises subjecting the magnet to the magnetizing field, and causing relative angular motion between the magnet and the magnetizing field within an angle  $\theta$  of  $\pm 45^\circ$  between a predetermined direction of magnetization and the direction of the applied magnetizing field.

35

\* \* \* \* \*

40

45

50

55

60

65

70

75